

## UNITED STATES PATENT OFFICE

HARRY M. ULLMANN AND EDWIN R. THEIS, OF BETHLEHEM, PENNSYLVANIA

## PROCESS OF UNHAIRING HIDES AND SKINS

No Drawing.

Application filed December 26, 1928. Serial No. 328,619.

This invention relates to a process of unhauling hides and skins involving the use of the pancreatic enzymes. For brevity in the following description only hides will be referred to, it being understood that animal skins generally are meant unless otherwise indicated. The unhauling of hides, i. e., the skins of large full grown animals, such as steer hides, is the principal application of the invention. Also for the sake of brevity only pancreatin will be referred to, it being understood that the material known as trypsin, a commercial concentrate of the proteases of the pancreas, or any other material containing pancreatic enzymes may be used.

Pancreatin has long been used as a bating agent and attempts have been made to use it as an unhauling agent but such attempts, so far as we are aware, have not resulted in a commercially successful process. For instance, it has been proposed to subject hides to be unhaired to a preliminary swelling in an acid or alkaline solution and thereafter to subject the hides to the action of pancreatin until unhauling occurs, that is, until the hair can be removed, for instance by sliding a finger over the hide. This treatment, however, works an undesirable degenerative and destructive action upon the hide, including digestion of the derma.

Our process is, in a sense, a modification of the so-called liming process. It is not designed to and does not eliminate liming but has the advantage that it greatly shortens the customary lime treatment. In the customary liming process cured hides are first soaked in water for about 24 hours to remove salt and are then put into a solution of lime for about 120 hours, more or less, depending upon the kind and condition of the hide and other factors after which the hair may be removed in the known way. It will be understood that our process as described is adapted to the treatment of cured or salted hides, although it readily may be modified and adapted to the treatment of fresh or uncured hides.

According to the process of our invention, 50 the cured hides are not subjected to any pre-

liminary swelling in acid or alkali nor to a preliminary and independent soaking as in the well-known liming process but the pancreatin is added directly to the water used for soaking the hides. Thus it may be considered that the customary soaking is replaced by a treatment with pancreatin or more logically that the treatment with pancreatin is superimposed upon or combined with the customary soaking. It is desirable, although not essential, that the pancreatin be added at the beginning of the soaking. The soaking in the presence of pancreatin is continued for about the customary length of time, say 20 hours, (this period of time may vary with the condition, cure and kind of hide, the temperature of operation, the concentration and activity of the pancreatin in the bath, etc.) and the hide is then transferred to the customary liming liquor where it is left for only a comparatively short time, say 20 hours, after which it is ready for the usual mechanical treatment for removing the loosened hair. It is noted that the hide is not left in the pancreatin-containing soaking bath until unhauling occurs, i. e., until the hair may be removed by sliding a finger over the hide. Indeed the hair should be still tight at the end of the soaking treatment. Due to the great variation in hides, it is impossible to specify precise conditions for the treatment of all hides. We prefer for the sake of economy to use a dilute solution of pancreatin for the combined pancreatin and soaking treatment, for example .02% to .04% of pancreatin based on the weight of the soaking water or solution. Higher concentrations of pancreatin up to say 0.1% may be used with a shortening of the treatment. The concentration of pancreatin in the soaking solution may vary from a minimum effective quantity, the lower limit apparently being in the neighborhood of .01%, up to that quantity which in a given time will deleteriously affect the hide. For example, a 1% solution acting upon steer hide at 70° F. for 20 hours ordinarily detrimentally affects the hide.

The temperature, about 60° F. to 80° F., and other conditions observed in the modi-

fied soaking and liming operations are the same as those used in the customary soaking and liming operations, the only variations being those referred to above, i. e., that the soaking water has pancreatin added to it and the soaking operation is limited, if necessary, to avoid detrimental action upon the hide, it being unnecessary to loosen the hair by the action of the pancreatin in the soaking bath, and the liming treatment is limited to a time sufficient to loosen the hair—the usual effect of liming.

10 The treatment described does not result in any appreciable degeneration of the derma of the hide. Net gains in hide due to hydration and the amount and quality of the finished leather are normal as compared with the product obtained by the known soaking and liming process.

15 20 We claim:

1. Process of unhauling hides which comprises soaking the hides in water containing pancreatin and thereafter liming the soaked hide.

25 2. Process of unhauling hides which comprises contacting the hides with a solution of pancreatin for a substantial period of time insufficient to produce unhauling and thereafter treating the hides with a solution of lime until the hair is loosened.

30 3. Process of unhauling hides which comprises soaking cured hides in the presence of pancreatin in quantity amounting to from about .02% to 0.1% of the soaking liquid for 35 a substantial period short of time sufficient to produce unhauling and thereafter subjecting the hides to a short liming treatment.

40 4. Process of unhauling hides which comprises soaking cured hides in the presence of pancreatin in quantity amounting to from .02% to .04% of the soaking liquid for about 20 hours at a temperature of from 60° F. to 80° F. and thereafter liming the hides for about 20 hours.

45 45 In testimony whereof, we affix our signatures.

HARRY M. ULLMANN.  
EDWIN R. THEIS.